

## UNITED STATES PATENT OFFICE

2,103,819

MANUFACTURE AND USE OF WETTING  
PREPARATIONS

Heinrich Lier, Basel, Switzerland, assignor to  
the firm of Chemical Works, formerly Sandoz,  
Basel, Switzerland

No Drawing. Application August 20, 1935, Se-  
rial No. 37,101. In Switzerland August 24,  
1934

4 Claims.

(Cl. 8—20)

I have found that naphthenic acids, if mixed in suitable proportions with hydrocarbons or such derivatives of hydrocarbons which resemble in their behaviour hydrocarbons are rendered soluble or more soluble in strong alkaline lyes, for instance mercerizing lyes. In order to obtain clear lyes of high efficacy a further addition of phenols may be necessary in special cases.

When added to alkaline lyes in very small quantities, these mixtures impart to them durable wetting-out properties, so that it is possible to mercerize dry raw and even sized cotton fibres very rapidly and to obtain a very high lustre in a single treatment.

In order to obtain the wetting preparations, raw or purified naphthenic acids obtainable from naphtha of any origin by the usual purification processes or any other treatment or fractions of such naphthenic acids are mixed with saturated or unsaturated hydrocarbons of the aliphatic, alicyclic, araliphatic or aromatic series, containing at least six carbon atoms in their molecule. These hydrocarbons may be partially or totally replaced by water-insoluble ethers or water-insoluble mono- or polyhalogenated hydrocarbons or halogenated ethers, all of them containing at least six carbon atoms. Suitable compounds are for instance petroleum hydrocarbons, benzine fractions, common petroleum, paraffin-oil, gas-oil, naphthenic hydrocarbons, oil of turpentine, dipentene, eucalyptus oil, oil of camphor, completely or partly hydrogenated aromatic hydrocarbons, aromatic hydrocarbons of the benzene, naphthalene and anthracene series, halogen substituted hydrocarbons (halogenated paraffin-oil, the products resulting from the action of chlorine or bromine upon olefines, mono- or polyhalogenated benzene and their homologues).

Suitable ethers are for instance diisoamylether, ethers of phenols without free hydroxyl groups, ethers of halogenated phenols.

Phenols which are needed to render the preparations completely soluble especially in strong lyes are phenol and its homologues for instance cresols, particularly meta- and para-cresol, mixtures of cresols, xylenols, mixtures of cresols and xylenols, ethylphenols, carvacrol, phenols, obtainable in the refining of charcoal tars, phenols, of low temperature tar or fractions therefrom, synthetic derivatives of phenols for instance sulphurated phenols, guaiacol, monoalkylethers of resorcin, naphthols; halogen substituted products of phenols as for instance para-chloro-phenol, technical mixtures of mono-chlorinated

cresols, orthochlorometacresol, orthochloropara-cresol, parachlorometacresol, brominated cresols and the like or any mixtures of all these different phenols.

The following examples, without being limitative, illustrate the new process and its technical application.

## Example 1

To a mercerizing lye of 30° Bé. are added 0.5 parts (by volume) of a mixture, consisting of 75 parts of a fraction of naphthenic acids (acid value=361), boiling between 130 and 140° C. under a pressure of 15 mm. and 25 parts of a technical mixture of petroleum hydrocarbons, boiling from 210—290° C. After good stirring the lye becomes completely clear and possesses an extraordinary high wetting power for raw cellulosic fibres or raw sized cotton fabrics.

Raw cotton pearl yarn (Maco 3/2) shrinks in 15 seconds 22 per cent of its origin length, whereas in presence of 0.5 parts (by volume) of the same naphthenic acid fraction and no petroleum hydrocarbon the shrinkage is only 1.6 per cent and this lye is troubled by separations of the insoluble alkali salt of the naphthenic acid.

Compared with commercial wetting agents for mercerizing purposes a contraction of 22 per cent in 15 seconds results only by adding 1.5 parts (by volume) of them.

The wetting-out capacity of the lye containing the new composition of matter remains unchanged a very long time, even if the lye has been kept uncovered.

In this mixture the petroleum hydrocarbon can be replaced by cymene, camphor-oils, hydrogenated naphthalenes as for instance tetra- or decahydronaphthalene, oil of turpentine, o-ethylated phenols from low temperature tar monochlorobenzene, chlorinated paraffin-oil or the like.

## Example 2

To mercerizing lyes of 33—35° Bé. are added 0.5 parts (by volume) of a fraction of technical naphthenic acid (acid value=400), boiling from 120—125° C. under a pressure of 14 mm. After good stirring, the lyes remain troubled and possess only a small wetting-out action. If 7 parts of the said fraction of naphthenic acid are mixed with 3 parts of cymene and 0.5 parts by volume of the mixture is added to the lyes, they become completely clear and show a much higher wetting-out action.

## Example 3

A mercerizing lye of 25° Bé. which contains 0.8

per cent (by volume) of a mixture of 62.5 parts of technical naphthenic acid (acid value=237), and 17.5 parts of petroleum hydrocarbons as in Example 1 is clear and possesses a high wetting-out action for raw yarns and raw wood cellulose. This high action remains unchanged, when the lye is kept for 4 days in an uncovered container. The special petroleum hydrocarbon can be replaced by common petroleum or gas-oil.

### Example 4

A mixture, containing 46 parts of a North-American petroleum naphthenic acid (acid value=306), boiling between 100-160° C. under 15 a pressure of 14 mm., 8 parts of technical de-cahydronaphthalene and 46 parts of a technical xylenol mixture is clearly soluble in a mercerizing lye of 30° Bé.

The shrinkage of a raw cotton pearl yarn (Maco 3/2) in a lye of 30° Bé., containing 1 per cent by volume of this mixture in only 30 seconds is 26 per cent of the origin length. A similar action and solubility results if the decahydro-naphthalene is replaced by monochlorobenzene, technical cymene, anisol, diisoamylether or the like.

*Example 5*

4 parts by volume of a technical xyleneol mixture are mixed with 3.7 parts of the petroleum hydrocarbon mentioned in Example 1 and 13.3 parts of commercial naphthenic acid.

8 parts of the mixture are introduced into 1000 parts of caustic soda solution of 28° Bé. in such a manner that at first only a small quantity of the lye is stirred with the mixture. The resulting solution is then mixed together with the remaining part of the lye.

40 The wetting action of the clear solution thus obtained is so great, that raw dry cotton fabrics as for instance raw sized Pipeline tissues are completely impregnated in a few seconds and shrink very rapidly. The thus obtained tissue is uniformly mercerized and possesses a very high lustre.

*Example 6*

50 A mixture of 72 parts of a technical mixture of liquid monochlorocresols, 8 parts of monochlorobenzene and 20 parts of a fraction of American naphthenic acid (acid value=273), boiling between 160-170° C. under a pressure of 14 mm. is clearly soluble in caustic soda solutions of 32 to 35° Bé, and impart to them a very high wetting-out power.

*Example 7*

5 parts by volume of low temperature tar phenols, boiling from 200-290° C., are mixed with 3.4 parts of the petroleum fraction used in Example 1 and 11.6 parts of the technical naphthenic acid used in Example 5.

A mercerizing lye of 28° Bé. which contains 0.75 parts by volume of this composition is com-

pletely clear and impregnates immediately raw dry cotton tissues or yarns.

### Example 3

0.8 per cent by volume of a mixture of 32.5 parts of technical xylenols, 17.5 parts of tetrahydronaphthalene and 50 parts of the naphthenic acid mentioned in the foregoing Example 7 are added to a mercerizing lye of 28° Bé. The action of this lye is much higher than that of a lye of 28° Bé. containing 1.6 per cent by volume of the mixture of 90 parts of technical xylenols, 5 parts of tetrahydronaphthalene and 5 parts of naphthenic acid, described in Example 10 of U. S. patent specification No. 1,998,550.

Shrinking tests show that in the first lye the contraction of raw dry cotton pearl yarn (Macc 3/2) amounts after 15 seconds to 21.4 per cent of the origin length, compared to 7.4 per cent in the other lye.

Both lyes contain the same substances, but not in the same proportions; the new mixture, containing much more of the hydrocarbon and less of the xylenols, possesses more than the double activity of the lye according to U. S. A. Patent No. 1,998,550.

### Example 9

A caustic potash solution of 30° Bé., containing 0.5 per cent by volume of a mixture of 46 parts of technical tar xyleneols, 3 parts of cymene and 46 parts of American naphthenic acid mentioned in Example 4 is clear and possesses a high wetting-out action.

The shrinkage of a raw dry cotton pearl yarn (Maco 3/2) in 15 seconds is 20.8 per cent of the origin length. 35

What I claim is:—

What I claim is.—

1. The alkaline mercerizing solutions possessing high wetting action and containing a mixture consisting of 95-50 per cent of naphthenic acids and of 5-50 per cent of organic compounds with at least six carbon atoms selected from the class consisting of saturated and unsaturated aliphatic, alicyclic, araliphatic and aromatic hydrocarbons and their water-insoluble ethers and their non-phenolic halogenated derivatives.

2. The alkaline mercerizing solutions possessing high wetting action and containing a mixture consisting of 75 per cent of naphthenic acids with acid number 361 and 25 per cent of a technical mixture of petroleum hydrocarbons boiling between 210° and 290° C. 50

3. The alkaline mercerizing solutions possessing high wetting action containing a mixture consisting of 80 per cent of naphthenic acids and of 20 per cent of monochlorobenzene. 55

and of 30 per cent of monochlorobenzene.

4. The alkaline mercerizing solutions possessing high wetting action and containing a mixture consisting of 70 per cent of naphthenic acids 60 and of 30 per cent of cymene.

HEINRICH LIEB